

# United States Patent Office

2,781,284

Patented Feb. 12, 1957

1

2,781,284

## GRAPHITIC HIGH CARBON-HIGH VANADIUM STEELS

Paul R. Borneman and Leonard V. Klaybor, Dunkirk, N. Y., assignors to Allegheny Ludlum Steel Corporation, Brackenridge, Pa., a corporation of Pennsylvania

No Drawing. Application November 9, 1955,  
Serial No. 545,993

4 Claims. (Cl. 148—31)

This invention relates to improvements in die steels and in particular to die steels containing graphite and high percentages of vanadium.

In the past many die steels have been made and used in applications for cold working dies and the like, notably among which are the die steels containing approximately 0.8% to 4.0% carbon, 3.0% to 15% vanadium, 0.2% to 2.0% chromium, 0.25% to 2.0% molybdenum and/or tungsten and the balance substantially iron. These steels have exhibited superior resistance to abrasion, galling, scoring and scuffing when used in such applications as cold working dies or liners for brick molds. These steels, however, have an inherent difficulty in that high percentages of the carbide forming elements such as chromium, molybdenum, tungsten and particularly vanadium are required for the steel to obtain the requisite abrasion resistance. This has resulted in the steels possessing high percentages of the carbides of the respective elements with the result that each incremental increase in the carbides present in the structure of these steels has produced a corresponding decrease in the machinability of said steels.

An object of this invention is to provide a steel having a high resistance to abrasion and containing graphitic carbon, which steel possesses a controllable hardenability and excellent machinability characteristics.

A more specific object of this invention is to provide a steel containing carbon, silicon, manganese, chromium, tungsten, molybdenum, vanadium and the balance iron having a high percentage of carbides and sufficient graphite for the steel to possess excellent machinability.

These and other objects of this invention will become apparent when read in conjunction with the following description.

In its broader aspects the steel of this invention comprises from about 1.5% to about 5.0% carbon, from about 1.4% to about 2.4% silicon, from about 1.10% to about 3.0% manganese, up to about 1% maximum chromium, up to about 1% maximum tungsten, up to about 1% maximum molybdenum, from about 3.0% to about 15.0% vanadium and the balance iron with incidental impurities.

The steel of this invention may be made and produced by any of the well-known steel mill practices, for example, electric arc furnace melting. Predetermined quantities of scrap and/or hot metal are placed in the furnace and melted to form a molten metal bath usually with a slag covering thereon. The details of the melting and refining of such steels are well known in the art and need not be described herein. After the molten metal is refined to obtain the steel of the desired chemical analysis, it is tapped into a ladle from which the molten metal is cast into ingots of predetermined shape and size. Upon solidification the ingots may be processed in any of the well-known manners, for example, by forging, pressing, extruding or hot rolling.

More specifically, the process used in the fabrication of the steel of this invention consists of heating the ingots

2

of the desired analysis to a temperature in the range between 1925° F. and 2025° F. at which temperature they are forged. After sufficient forging to break and distribute the "as-cast" structure, the steel may be hot rolled in any desired manner to form the semi-finished mill product, for example, billets, bars and the like. The hot rolled steel is annealed by heating to a temperature above the critical temperature and thereafter slowly cooled to a temperature below the critical temperature. In practice, it is preferred to anneal the steel at a temperature between 1400° F. and 1550° F. and thereafter slowly cool the steel to about 500° F. The essential purpose of the annealing and the subsequent slow cooling is to promote the precipitation of graphite simultaneously with the spheroidization of the carbides. This results in the steel being graphitized and thereby imparts the desired free machining properties thereto. The steel can be machined to any desired shape from which it is heat treated to obtain the desired physical properties of hardness, strength and ductility.

The preferred heat treatment to develop the physical properties of the steel after graphitization consists of a solution heat treatment at a temperature in the range between 1600° F. and 1750° F. for a time period of about 5 minutes to 4 hours depending upon the size of the piece being heat treated and followed by quenching in oil. This results in the steel having a hardness of about 60 R<sub>c</sub> to 65 R<sub>c</sub>. The steel is then further heat treated by tempering at a temperature in the range between 300° F. and 1300° F. in order to increase the strength and ductility of said steel.

Reference may be had to Table I illustrating the chemical analysis of the general range, the preferred range, and steels A and AL-64 which are within the general range. It will be appreciated that in the following table where reference is made to iron comprising the balance of the steel, it is to be understood that the usual impurities found in such steels are also included, for example, not more than 1.5% of such elements as copper, cobalt, nickel, sulfur, phosphorus and the like.

TABLE I

Percent by weight

|            | General range  | Preferred range | Steel A | AL-64 |
|------------|----------------|-----------------|---------|-------|
| Carbon     | 1.5-5.0        | 2.90-3.10       | 3.18    | 2.90  |
| Silicon    | 1.4-2.4        | 1.60-1.90       | 1.95    | 1.89  |
| Manganese  | 0.10-3.00      | 1.0-1.2         | 0.13    | 1.16  |
| Chromium   | Up to 1.0 max. | 0.45 max        | 0.41    | 0.04  |
| Tungsten   | Up to 1.0 max. | 0.5 max         | 0.05    | 0.09  |
| Molybdenum | Up to 1.0 max. | 0.25-0.45       | 0.30    | 0.43  |
| Vanadium   | 3.0-15.0       | 7.75-8.25       | 8.02    | 8.25  |
| Iron       | Bal.           | Bal.            | Bal.    | Bal.  |
| Graphite   | 0.01-1.5       | 0.3-1.0         | 0.57    | 0.91  |

Each of the elements given hereinbefore in Table I performs a specific function and therefore each element is required to be maintained within the range given. Carbon in the amount between 1.5% and 5.0% is needed to form the desired carbides for imparting high abrasion resistance as well as sufficient excess carbon above the amount needed to form the carbides for the purpose of forming graphite for imparting the requisite machinability characteristics to the steel. It is preferred to maintain silicon in the range between 1.4% and 2.4% because silicon is the predominant element in this steel for promoting graphitization upon proper heat treatment. Manganese in the general range given imparts sufficient hot workability and provides the requisite deep hardenability. By controlling the amount of manganese present in the steel it is possible to control the amount of hardenability as will be described hereinafter. The complex carbide forming elements chromium, tungsten and molybdenum,

within the ranges given, contribute to both the hardenability and the hardness developed during heat treatment in addition to combining with a portion of the carbon to form carbides which contribute to the strength and abrasion resistance of the steel. Careful control of the amount of these elements present in the steel is necessary since each has an inhibiting effect on the formation of graphite and incremental increases in the amount of these elements present in the analysis will cause corresponding reductions in the amount of graphite which can be precipitated during annealing. Vanadium is the chief carbide forming element within the analysis of the alloy of this invention and combines with larger portion of the carbon to form carbides with the result that the steels show a high resistance to abrasion, galling, scoring and scuffing.

As a specific example of the steel of this invention, steel A was made with the analysis as given hereinbefore in Table I. Steel A was forged and thereafter hot rolled from a temperature of 1950° F. into bar form from which it was annealed at 1450° F. and slowly cooled therefrom. The annealing heat treatment and subsequent slow cooling caused the formation of spheroidal carbides within the microstructure with 0.57% carbon being present in the form of graphite. This steel was machined to the desired shape which was then solution heat treated by heating it at a temperature of 1675° F. for two hours followed by an oil quench. This hardening heat treatment resulted in steel A having a hardness of between 63 Re and 64 Re. After tempering at a temperature of 400° F. for 2 hours, said steel showed an increase in strength and ductility sufficient for use, for example, as a cold working die or as a liner for brick molds.

As was stated hereinbefore, manganese is essential to provide the requisite hardenability in the steel of this invention. This is more clearly illustrated by comparing the hardenability data of steels A and AL-64 listed in Table I. These steels have substantially similar compositions with the exception of manganese. Reference may be had to Table II which contains the test results obtained on a standard Jominy Test for measuring the depth of penetration of the hardness for steel A and steel AL-64.

TABLE II.—HARDENABILITY

| Distance from quenched end<br>in $\frac{1}{16}$ of an inch | Steel A | Steel AL-64 |
|------------------------------------------------------------|---------|-------------|
| 1                                                          | 63.5    | 63          |
| 2                                                          | 63.4    | 63          |
| 3                                                          | 63.0    | 63          |
| 4                                                          | 62.5    | 63          |
| 5                                                          | 60.2    | 62.5        |
| 6                                                          | 57.6    | 62.5        |
| 7                                                          | 52.7    | 62          |
| 8                                                          | 49.0    | 62          |
| 9                                                          | 48.0    | 61.5        |
| 10                                                         | 47.5    | 61          |
| 11                                                         | 46.9    | 60          |
| 12                                                         | 46.7    | 59          |
| 13                                                         | 46.0    | 59          |
| 14                                                         | 45.8    | 57.5        |
| 15                                                         | 45.2    | 56          |
| 16                                                         | 44.8    | 55          |
| 17                                                         | 44.2    | 52          |
| 18                                                         | 43.3    | 48          |
| 20                                                         | 42.7    | 44          |
| 22                                                         | 42.2    | 41          |
| 24                                                         | 41.3    | 39          |
| 26                                                         | 40.8    | 38          |
| 28                                                         | 40.7    | 36.5        |
| 30                                                         | 40.3    | 36.5        |
| 32                                                         |         |             |

As is evident from Table II, increasing the manganese content to about 1% increases the depth of penetration or hardness as measured at the 50% martensite point from about  $\frac{1}{16}$  for steel A to about  $\frac{1}{4}$  in steel AL-64. It is clearly evident that where deeper hardenability is desired the manganese content should be at least 1% and preferably it should be maintained near the higher end of the preferred range given hereinbefore in Table I.

The steel of this invention has excellent machinability which can be demonstrated relatively by sawing with a power hacksaw. The power hacksaw test consists of cutting two-inch square billets under identical conditions. In this test the billets are sawed on a power hacksaw using a new molybdenum type high speed steel blade. After the initial cut is made, the material is advanced and a second cut is made. The speed or downward feed of the power hacksaw is increased in each succeeding cut to increase the severity of the test until the point is reached where the blade shows excessive wear or breaks, whichever occurs first. The number of cuts and the relative speeds of the saw in each cut compared to the number of cuts and the relative speed for the hacksaw blade in the standard or comparative steel gives a measure of the relative machinability of the steels.

In applying the above described test to determine the relative machinability of the steel of this invention as compared to another steel having the same degree of resistance to abrasion, galling, scoring and scuffing in the hardened state, a steel having the following analysis was used as the standard: about 2.91% carbon, about 0.37% manganese, about 0.35% silicon, about 0.11% tungsten, about 0.90 chromium, about 0.96% molybdenum, about 10.45 vanadium and the balance iron with incidental impurities. The standard steel was hot worked into a two-inch square billet which was annealed to a hardness of about 269 BHN. Metallographic and wet chemical analysis failed to show the presence of graphite in the standard steel in the annealed condition. Steel AL-64 having the analysis given hereinbefore and in the form of a two-inch square billet was then compared to the standard steel, it being noted that steel AL-64 had about 0.91% graphite after annealing at 1450° F. and a hardness of 269 BHN.

Steel AL-64 was subjected to five successive cuts across the section of the two-inch billet using a new molybdenum type high speed steel blade having 6 teeth per inch with the speed of the blade being increased with each successive cut. After the fifth cut, the blade showed some wear and the cutting was stopped on steel AL-64. After an identically new hacksaw blade was inserted in the power hacksaw, the standard steel of the analysis given hereinbefore was sawed in the same manner as steel AL-64. The speed of the hacksaw was adjusted so that substantially the same speed was used for each cut on the standard steel as was used on the same numbered cut on steel AL-64. It was found that after the first cut through the standard steel, the blade showed some wear, and before the second cut could be completed, the saw blade broke. It is significant to point out that the speed of the saw blade was more than twice as fast during the fifth cut on steel AL-64 as compared to the speed of the saw blade during the second cut on the standard steel which broke the blade. It is evident from the above described test that the steel of this invention possesses a superior machinability to that of comparable steels having substantially the same resistance to abrasion, galling, scoring and scuffing. It is believed that the superior machinability has been achieved by the graphite which is present through a critical proportioning of the alloying elements cooperating with the heat treatment given hereinbefore to promote graphitization, thereby imparting the requisite machinability properties thereto.

There are no special techniques, processing or equipment used in the production of this steel in order to obtain the desired characteristics. In addition, there is a noticeable absence of strategic and costly alloying elements, thus making the steel valuable from the economical aspect.

We claim:

1. An iron alloy possessing excellent machinability characteristics, superior resistance to abrasion, scoring, scuffing and galling and controllable hardenability and consisting of, from about 1.5% to about 5.0% carbon, from about 1.4% to about 2.4% silicon, from about 0.10% to about 3.0% manganese, up to 1.0% chromium, up to

1.0% tungsten, up to 1.0% molybdenum, from about 3.0% to about 15.0% vanadium and the balance iron with incidental impurities, the alloy having from about 0.01% to 1.5% of carbon present in the form of graphite resulting from heat treatment at a temperature in the range between 1400° F. and 1550° F., and slowly cooling therefrom.

2. An iron alloy possessing excellent machinability characteristics and superior resistance to abrasion, scoring, scuffing and galling and consisting of from 2.90% to 3.1% carbon, from 1.60% to 1.90% silicon, from 1.0% to 1.2% manganese, up to 0.45% maximum chromium, up to 0.5% maximum tungsten, from 0.25% to 0.45% molybdenum, from 7.75% to 8.25% vanadium, and the balance iron with incidental impurities, the alloy having from about 0.3% to 1.0% of carbon present in the alloy in the form of graphite resulting from heat treatment at a temperature in the range between 1400° F. and 1550° F., and slowly cooling therefrom.

3. An iron alloy for use as a cold working die and containing about 3.18% carbon, about 1.95% silicon, about 0.13% manganese, about 0.41% chromium, about 0.05% tungsten, about 0.3% molybdenum, about 8.02% vanadium, and the balance substantially iron with incidental impurities, the alloy having about 0.57% of carbon present in the alloy in the form of graphite resulting from treatment at 1450° F. and slowly cooling therefrom.

4. An iron alloy for use as a cold working die and having a deep hardenability and containing about 2.90% carbon, about 1.89% silicon, about 1.16% manganese, about 0.04% chromium, about 0.09% tungsten, about 0.43% molybdenum, about 8.25% vanadium and the balance substantially iron with incidental impurities, the alloy having about 0.91% of carbon present in the alloy in the form of graphite resulting from heat treatment at 1450° F., and slowly cooling therefrom.

No references cited.